

## UNITED STATES PATENT OFFICE

2,351,468

## STABILIZED EXPLOSIVE COMPOSITION

Clifford A. Woodbury, Media, Pa., assignor to E. I.  
du Pont de Nemours & Company, Wilmington,  
Del., a corporation of Delaware

No Drawing. Application July 18, 1941,  
Serial No. 402,956

8 Claims. (Cl. 52—13)

This invention relates to a novel explosive composition adapted for use under extreme conditions of temperature and pressure.

For many years explosives have been used in the shooting of oil wells to start the flow of oil or to increase it after the wells have ceased to produce paying quantities. The explosive that has been most favored in such oil well blasting in the past has been liquid nitroglycerin, which has been loaded in the desired amount into special containers to form the well-known torpedoes for use. Another form of high explosive used in oil well blasting has been the so-called solidified nitroglycerin, or blasting gelatin, which consists of a thick viscous material resembling crude, translucent rubber, as a result of the solution of nitrocotton in nitroglycerin in the ratio of around 4 to 9 parts of nitrocotton to 90 parts of nitroglycerin.

Such explosives were generally satisfactory and reliable in the shooting of relatively shallow wells. At the present time, however, depths of 10,000 ft. to 15,000 ft. are encountered and at such depths the conditions are such that the foregoing explosives high in nitroglycerin are somewhat unreliable and hazardous unless unusual precautions are taken. Two factors come in to cause difficulties. In the first place, high pressures are met in deep hole shooting, of the order of several thousand pounds per square inch. Under such pressures, the explosives show erratic behavior. They may become insensitive and fail to shoot, or may explode prematurely. Either condition is undesirable, and the presence of unexploded, potentially explosive material in the bore hole becomes a hazard, since subsequent boring into the charge would probably prove disastrous. A second troublesome factor comes in the high temperatures resulting from deep drilling, for example, up to 200° F. and higher. Whereas it is frequently the practice, after an explosive charge has been lowered into a hole, to set the time bomb for 20 or more hours, explosion may take place prematurely in 4 or 5 hours under the high temperature and pressure conditions to which the charge is exposed. Such lack of reliability is hazardous, since tamping or cementing operations may be in progress at the time of the explosion.

An object of the present invention is an ex-

5 plosive composition adapted for deep well shooting and possessing improved reliability of performance and markedly increased stability. A further object is a stabilized explosive composition capable of withstanding excessive temperature and pressure conditions while maintaining its original explosive properties. Additional objects will be disclosed as the invention is described more at length hereinafter.

10 I have found that the foregoing objects are obtained by employing an explosive composition adapted for use in deep wells, and comprising more than 60% of nitroglycerin or other liquid explosive nitric ester and a suitable amount of a weak organic base as stabilizer therefor. Preferably, the explosive will contain more than 90% of nitroglycerin, and may comprise either liquid nitroglycerin, or a blasting gelatin type.

15 As stated above, a weak organic base is included as a stabilizing ingredient in the explosive composition, and I find it essential that the base be one having a dissociation constant lower than  $1 \times 10^{-6}$  since too strong a base might have a decomposing effect on the nitroglycerin or other liquid nitric ester present. Such bases are capable of serving as acid acceptors in case of decomposition of the nitric ester. The following will serve as illustrations of organic bases that fall within the scope of the invention. I 20 find it preferable to use an amount of the organic base within the range of 0.5 to 5.0% of the explosive content:

|    | Base                            | Dissociation constant |
|----|---------------------------------|-----------------------|
| 35 | Urea.....                       | $1.5 \times 10^{-14}$ |
|    | Alpha-naphthylamine.....        | $9.9 \times 10^{-11}$ |
|    | Beta-naphthylamine.....         | $2 \times 10^{-10}$   |
|    | Pyridine.....                   | $3.3 \times 10^{-9}$  |
|    | Phenylenediamine.....           | $3.3 \times 10^{-10}$ |
| 40 | o-Toluidine.....                | $3.3 \times 10^{-10}$ |
|    | Diphenylamine.....              | $<1 \times 10^{-14}$  |
|    | Sym-diphenyl-dimethyl urea..... | $<1 \times 10^{-14}$  |
|    | Sym-diphenyl diethyl urea.....  | $<1 \times 10^{-14}$  |
|    | Thiourea.....                   | $1.1 \times 10^{-13}$ |
|    | Acetanilid.....                 | $4.1 \times 10^{-14}$ |
| 45 | Dicyandiamid.....               | $<1 \times 10^{-14}$  |

While the foregoing weak bases are all applicable under the invention, I find that diphenylamine and the diphenyl-dialkyl ureas are particularly advantageous. The following examples will serve to illustrate the stabilizing effect of

such compounds when used with nitroglycerin or blasting gelatin at elevated temperatures and pressure. The effect of the stabilizer is shown by the increased time in minutes elapsing before the explosion of the charge in question, this increase being the result of the presence of the added compound:

5 introduced into the composition at the time of manufacture. It will be understood that, in addition to nitroglycerin, the invention is applicable to solutions of other materials in nitroglycerin, for example, nitroglycerin containing ethylene glycol dinitrate, or other desired material. The liquid explosive may also be com-

| Explosive                     | Stabilizer                       | Amt.    | Pressure     | Temperature                                        |                                           |
|-------------------------------|----------------------------------|---------|--------------|----------------------------------------------------|-------------------------------------------|
|                               |                                  |         |              | 212° F.                                            | 275° F.                                   |
| Nitroglycerin                 | None                             | Percent | Lbs./sq. in. | Mins.                                              | Mins.                                     |
|                               | do                               |         |              |                                                    |                                           |
|                               | Diphenylamine                    | 2       |              | 1,500<br>3,000<br>1,500<br>3,000<br>1,500<br>3,000 | 157<br>82<br>>360<br>>300<br>>300<br>>330 |
|                               | Diphenyldiethylurea              | 2       |              | 17<br>9<br>97<br>73<br>80<br>39                    | 17<br>9<br>97<br>73<br>80<br>39           |
| Blasting gelatin <sup>1</sup> | (None)<br>(Diphenyldimethylurea) | 2       | 3,000        | >330                                               | 72                                        |

<sup>1</sup> 91% nitroglycerin, 4.5% nitrocotton, 3.5% wood pulp, 1.0% chalk.

In the foregoing tabulation, the time is given in minutes which elapsed before the spontaneous explosion of the charge in each case, under the temperature and pressure conditions shown. From these results, it will be seen that the organic bases have a very considerable stabilizing effect. For example, in the case of liquid nitroglycerin, the presence of 2% of diphenylamine increased the life of the explosive at 3000 lbs./sq. in. and 275° F. from 9 to 73 minutes; while at 212° F., under the same pressure, the time was increased from 82 to over 300 minutes. Likewise, at 1500 lbs./sq. in., the introduction of the same amount of diphenylamine increased the life from 157 to more than 360 minutes at 212° F., while the increase under the same pressure at 275° F. was from 17 to 97 minutes. Similar stabilizing effects were obtained by the use of other weak bases of the type specified. It will be understood that the conditions of testing shown in the examples are somewhat more severe than would be expected under field conditions, but the same stabilizing effect would result.

It has been stated that the preferred amount of weak base for use as stabilizer is preferably within the range of 0.5 to 5.0%, based on the weight of the explosive compound. A smaller amount than 0.5% is insufficient to give the desired effect, while the use of more than 5% of such material would lower the strength of the explosive compound, by the introduction of so much non-explosive material. Since the base will be largely dissolved in the nitroglycerin also, its presence would tend to desensitize the composition, if too large an amount were used.

In using the stabilizing materials described, they will desirably be dissolved in the nitroglycerin some time before use in order to insure solution and prevent segregation. In the case of the liquid nitroglycerin, diphenylamine or other organic base can be introduced into the container in increments, if desired, and the liquid explosive be poured in in the same manner. When blasting gelatin is used, the base should be in-

posed entirely, if desired, of the above nitroglycerin or any other suitable liquid explosive nitric ester.

It should be noted that it is not part of my invention to include these organic bases in commercial dynamite compositions.

The invention has been described in the foregoing at some length. It will be understood, however, that many variations may be introduced in the specific materials used and in amounts without departure from the scope of the invention. I intend to be limited therefore only by the following patent claims.

I claim:

1. An oil well explosive composition comprising more than 60% of a liquid explosive nitric ester and between 0.5 and 5.0% of an organic base having a dissociation constant lower than  $1 \times 10^{-5}$ .

2. An oil well explosive composition comprising more than 90% of a liquid explosive nitric ester and between 0.5 and 5.0% of an organic base having a dissociation constant lower than  $1 \times 10^{-5}$ .

3. An oil well explosive composition comprising more than 60% of nitroglycerin and between 0.5 and 5.0% of an organic base having a dissociation constant lower than  $1 \times 10^{-5}$ .

4. The explosive composition of claim 3, in which the organic base is diphenylamine.

5. The explosive composition of claim 3, in which the organic base is a substituted urea.

6. The explosive composition of claim 3, in which the organic base is a diphenyl-dialkyl urea.

7. An oil well explosive composition adapted for use in deep wells comprising more than 90% of a liquid explosive nitric ester and between 0.5 and 5.0% of diphenylamine.

8. An oil well explosive composition adapted for use in deep wells comprising more than 90% of a liquid explosive nitric ester, sufficient nitrocellulose to form a firm gel with the liquid nitric ester, and between 0.5 and 5.0% of a diphenyl-dialkyl urea.

CLIFFORD A. WOODBURY.